

**1**

3,488,264

**HIGH SPEED ELECTRODEPOSITION OF NICKEL**  
Raymond E. Bailey, Mentor, and Arthur H. DuRose,  
Richmond, Ohio, assignors to Kewanee Oil Company,  
Bryn Mawr, Pa., a corporation of Delaware  
No Drawing. Continuation-in-part of application Ser. No.  
443,077, Mar. 26, 1965. This application Sept. 27, 1968,  
Ser. No. 763,409

Int. Cl. C23b 5/08, 5/46

U.S. Cl. 204—49

9 Claims

**ABSTRACT OF THE DISCLOSURE**

A process for the high speed electrodeposition of nickel comprising electrodepositing nickel on a cathode while employing an insoluble anode from a chloride and bromide free bath consisting essentially of an aqueous solution of nickel ions having a pH within the range of 2.0 to 4.5 and containing a 1,2-benzopyrone compound, during said electrodeposition said bath being rapidly passed over said cathode at a current density of at least 500 amperes per square foot and at a temperature of at least 150° F.

This application is a continuation-in-part of application Ser. No. 443,077 filed Mar. 26, 1965, now abandoned.

The present invention relates to high speed electrodeposition of nickel, cobalt, or nickel-cobalt alloys. More particularly, the invention relates to an improved process for such electrodeposition whereby smooth lustrous nickel, cobalt, or nickel-cobalt alloy is deposited on a cathode at very high current densities and temperatures while avoiding a brittle deposit.

The great majority of conventional processes for electrodepositing nickel, cobalt or nickel-cobalt alloy have refrained from utilizing high current densities despite some practical advantages, such as faster plating. Depending upon the composition of the plating bath, current densities of 200 amperes per square foot or higher have resulted in so-called "burning"; that is, the production of nickel hydrate at the cathode. Concentration polarization is associated with such high current densities under these conditions; and whatever the cause may be, the nickel deposit has been commercially unacceptable.

Attempts to utilize higher current densities more satisfactorily have included the use of plating baths operated at unusually high temperatures, as well as baths which contain higher conducting solutions. In particular, it has been suggested that the chloride content of the bath should be markedly increased or even that an all-chloride bath should be employed to assist in the use of such high current densities—see "High Speed Nickel Plating," Pinner & Kinnaman, Monthly Review, Amer. Electropolastics Assoc., 32, 227-34 (1945). Such baths, particularly when operated at high temperatures, have not proved at all satisfactory. If insoluble anodes are used, chlorine is given off, and will, of course, attack the anode as well as the plating equipment, and since it is a poisonous gas it must be removed from the area. Furthermore, the nickel deposited from such a bath is exceedingly fine grained and although it tends to be quite hard, it also tends to be quite brittle.

Attempts to utilize a very high current density with other types of baths, particularly all-sulfate baths, have overcome some of these objections but also have been

**2**

unsatisfactory. An all-sulfate bath will produce a very coarse grained nickel deposit which tends to be more ductile than that deposited from the chloride-containing bath. But it has been very rough and not sufficiently ductile to be wholly satisfactory. In this connection, it has been observed that for the all-sulfate bath, if the pH is increased, the ductility of the nickel deposit is decreased. Thus, it has been considered necessary to use a low pH which, of course, presents difficulties.

Thus, no matter what general type of bath is employed, it is a most difficult problem to secure very high current densities under practicable plating conditions and still maintain the bath properly while producing the desired properties in the nickel deposit. In fact, these results cannot be obtained without considerable agitation in the bath since it is necessary to provide a high rate of flow of the electrolyte over the cathode surface. Theoretically, the limiting current density for a sound nickel deposit increases with rate of flow of the electrolyte. There are, of course, many practical difficulties. In addition to some discussed above, these include the high voltage needed, overheating of the electrolyte, the difficulties of anode to cathode spacing, and the problems caused by failure to maintain uniform flow of the electrolyte.

The electrodepositing of bright or semibright nickel under high current densities and high temperature conditions while at the same time obtaining a deposit which is satisfactory as to ductility, smoothness, and adhesion presents a particularly difficult problem. Addition agents incorporated into a bath to provide a bright or semibright deposit, or to act as levelers; that is, to provide a smoother surface and to assist in hiding small imperfections in the basis metal, or both, are rendered much less effective, or in some cases completely ineffective, by the conditions of a high speed plating process. In fact, it has been stated by one authority, Clauss—"A Study of Variations in Certain Characteristics of Bright Nickel Deposits With Variations in Bath Temperature," Technical Proceedings, American Platers Society (1960), pp. 105-109, "this investigation of organic addition agents certainly shows that satisfactory bright nickel deposits may be obtained at high temperatures but the efficiencies of existing useful compounds is decidedly low when compared with the effectiveness at normal plating temperatures." It should be noted that this investigation did not utilize high current densities or high flow rates of the electrolyte; but the author noted, which has been our observation, that many common brighteners are rendered most ineffective or are completely destroyed by hot plating baths, particularly those depending upon unsaturation for their effectiveness. The use of such addition agents is surely most desirable if bright or semibright nickel is to be obtained and they are most desirable in order to produce a grain structure of the desired type. They also should assist in producing a smooth surface; that is, they should provide some appreciable leveling effect or at least not interfere with the leveling otherwise obtainable. Under the conditions of the high speed plating process, it has not proved possible heretofore to provide addition agents capable of gaining those desired results although some have aided in one way or another to some extent.

The addition agents contemplated by the present invention, contrary to expectations, were found to enhance the brightening and leveling of the nickel deposit as compared with such effects in a conventional nickel plating

process despite the very high current densities and temperatures, as well as the high flow rate of the electrolyte across the cathode. In fact, in some instances, it has proved possible to produce a fully bright nickel deposit from a bath by utilizing these very high current densities. Contrary to expectations, the desired concentration could be maintained readily in the bath without undue loss, while obtaining a deposit of satisfactory ductility and smoothness.

Inasmuch as it is a necessary part of the present high speed plating process to obtain a high flow rate of the electrolyte, it is most desirable that contoured insoluble anodes be employed. Such anodes make it easier to provide a uniform but minimum spacing between the anode and the cathode so that more uniform current densities may be maintained across the cathode. While this result is always desirable, it is especially important in the present process in view of the high current densities employed. In addition to the substantial saving in time, this process also saves nickel since it has been shown that the recessed areas of the cathode or other parts of the cathode which would normally have a low current density, can be plated more readily. Thus, it is not necessary to build up the thickness of the plate in high current density areas to such a marked extent as is done in conventional processing.

Broadly, the instant invention comprises a high speed process for the electrodeposition of nickel, cobalt, nickel-cobalt alloy wherein the metal is deposited from a chloride and bromide free bath which employs insoluble anodes. The bath is maintained at a pH in the range of 2.0 to 4.5. Coumarin or a substituted coumarin is present as an addition agent in the bath. The bath of the instant invention is operated at a temperature of at least 150° F. utilizing current densities of at least 500 amperes per sq. foot. The electroplating bath of the instant invention must also be subjected to high agitation during plating with the minimum agitation being a flow rate past the cathode of at least 300 feet per minute. Each of the above mentioned essential aspects of the instant invention will be discussed in detail in the remainder of the specification.

In the practice of the present invention, the electroplating bath composition can be varied extensively so long as the bath is maintained substantially free of chloride and bromide ions. Nickel salts such as nickel sulfate, fluoborate, acetate, sulfamate, perchlorate, and trichloroacetate may be used for supplying nickel to the solution. However, the all sulfate solution is preferred, and one substantially free of chloride. Lead anodes can be used with the sulfate solution but not when a substantial concentration of the other anions are present. During the electrolysis, nickel is deposited at the cathode and the pH decreases. The solution may be regenerated by the addition of basic nickel compounds, such as nickel hydrate, carbonate, or oxide. It may also be regenerated by use of nickel powder or electrolytic means in auxiliary equipment. Also, semipermeable membranes have been used. Later in the instant specification, a preferred embodiment will be discussed with respect to pH which permits the most economical regeneration of nickel baths useful in the instant invention.

During the practice of the instant invention, the temperature of the plating bath is maintained above 150° F., and preferably, although not necessarily, within the range of 180° F. to 210° F. As the current is applied, the plating solution is agitated very rapidly. This may be accomplished by various well-known means, but preferably the agitation is carried out by pumping the electrolytic solution over the surface of the cathode at a rapid rate, which is at least 300 feet per minute and preferably at least 600 feet per minute. When insoluble anodes are employed, a very small spacing can be used between the anode and the cathode thus making this high flow rate easier to obtain. It is desirable, however, that a substantially uniform flow rate be maintained at the surface of the cathode, and due to turbulence, eddying, and other fluid flow prob-

lems this may not be easily accomplished. It may even be necessary to place baffles at strategic points best learned through experience.

As stated previously, the current density in the practice of the instant invention must be greater than 500 amps per square foot. However, the maximum current density operable for a given plating operation is directly dependent on the rate of agitation or flow rate of the bath past the cathode. For example, if the flow rate past the cathode is maintained at 5 feet per second, the limiting current density in the practice of the instant invention is about 700 amps per square foot. At 22 feet per second the limiting current density is 3,000 amps per square foot whereas at a flow rate of 50 feet per second the limiting current density is 8,000 amps per square foot.

The use of insoluble anodes such as lead, carbon, graphite, platinum, platinized titanium, and lead alloyed with small amounts of tin, silver, or cobalt is a necessary part of the present invention and results in a particular advantage in the practice of the instant invention. Normally, insoluble anodes are never used in plating baths which contain organic additives, the reason being that such organic addition agents are rapidly consumed by anodic oxidation. Surprisingly, however, in the practice of the instant invention, it has been found that the anodic oxidation inherent in the use of insoluble anodes has a beneficial result in the practice of the instant invention. The coumarin or substituted coumarin addition agents used in the instant invention gradually breaks down at the cathode to form deleterious reduction products. However, these deleterious reduction products are controlled and maintained at a harmless level due to the anodic oxidation effected at the insoluble anode. The exact mechanism is not known with certainty but it is known that melilotic acid is formed and its harmful effects on the plating process are avoided whether it be by oxidation of the harmful acid at the anode which destroys side chains and gives off CO<sub>2</sub> or whether it polymerizes the melilotic acid so that the standard activated carbon treatment of such bath removes the same. Under ordinary plating conditions, the deleterious product formed at the cathode in baths containing a coumarin or derivative thereof will accumulate to a concentration from about 0.025 M and begins to have harmful effects at about 0.005 M. Under the high speed conditions of the instant invention utilizing insoluble anodes in a substantially chloride free bath, these deleterious reduction products are destroyed at the anode and accumulate to a concentration of only about 0.001 to 0.002 M.

Coumarin may be used as a leveling and brightening agent under the above described high plating speed conditions which involve high temperatures, high agitation rates, insoluble anodes, and chloride free nickel solutions. However, because of these conditions coumarin has a higher than normal consumption rate. Because of the high temperature, the volatilization of coumarin is higher than would be desired. Therefore, the use of leveling agents which have a lower electrolytic consumption rate and/or volatilization rate would be advantageous. We have found that certain 1,2-benzopyrone compounds have these properties. For example, the volatility of 3-chlorocoumarin is not appreciably less than that for coumarin but the electrolytic consumption rate is about 25% less than that for coumarin. Methyl-coumarin has about the same electrolytic consumption rate as coumarin but a lower volatility. Acetyl-coumarin has both a lower electrolytic consumption rate and lower volatility.

The substituent groups may be on either the aromatic ring or the heterocyclic ring of the coumarin molecule. The substituent groups may be halogen, acetyl, hydroxy, hydroxymethyl, hydroxyethyl, methoxy, ethoxy, acetamino, N-formylamino, propargyl, cyano, methyl, ethyl, dimethylamino, or diethylamino. Acidic substituents, such as carboxy, sulfonate, and sulfonamide groups are not

desirable except in very low concentration and in conjunction with the preferred compounds.

The preferred compounds have a boiling point greater than 290° C. and a melting point greater than 70° C. Table I sets forth a group of such compounds together with the concentration adapted to produce the best results. Another advantage of the preferred substituted benzopyrones is that they have a higher melting point than coumarin and, therefore, do not melt and float on the solution surface and cause problems by sticking to the surfaces of equipment.

TABLE I

| Substituted 1,2-benzopyrone—                    | Moles per liter |
|-------------------------------------------------|-----------------|
| (1) 3-chlorocoumarin (bromo, iodo, fluoro)----- | 0.0002-0.003    |
| (2) 3-acetylcoumarin-----                       | 0.0002-0.003    |
| (3) 6-acetylamino coumarin-----                 | 0.0002-0.002    |
| (4) 3-hydroxycoumarin-----                      | 0.0002-0.002    |
| (5) 3-cyanocoumarin-----                        | 0.0002-0.002    |
| (6) 3- or 4-methyl coumarin-----                | 0.0002-0.003    |
| (7) 6-methyl coumarin-----                      | 0.0002-0.003    |
| (8) 4,8-dimethylcoumarin-----                   | 0.0002-0.003    |
| (9) 7-diethylamino-4-methyl coumarin-----       | 0.0002-0.002    |
| (10) 6-hydroxycoumarin-----                     | 0.001-0.004     |
| (11) 6-(1-glucosaminio) coumarin-----           | 0.0002-0.002    |
| (12) 6-hydroxymethylcoumarin-----               | 0.0002-0.003    |
| (13) 8-hydroxyethylcoumarin-----                | 0.0002-0.003    |
| (14) 7-methoxycoumarin-----                     | 0.0002-0.003    |
| (15) 8-ethoxycoumarin-----                      | 0.0002-0.003    |

In order that those skilled in the art may better understand how the present invention may be carried into effect, the following examples are provided by way of illustration, but not of limitation. Unless otherwise specifically indicated all temperatures are in degrees centigrade and all parts and percentages are by weight.

## EXAMPLE I

Two solutions containing 50 ounces per gallon of nickel sulfate and 6 ounces per gallon of boric acid were stirred uniformly at a temperature of 185° F. One solution contained 0.0004 mole per liter of coumarin and the other 0.0004 mole per liter of 3-chlorocoumarin. The solution surface area was 27 square inches. The loss of coumarin by volatilization was 0.001 mole per liter per 1,000 hours and the loss of 3-chlorocoumarin was 0.0008 mole per liter per 1,000 hours. When the solution was electrolyzed at 1,000 amperes per square foot, the consumption rate of chlorocoumarin was markedly less than that of coumarin, being at least 25 percent less.

Using the above solution but employing instead of 3-chlorocoumarin, the compounds numbered 2, 3, and 8 of Table I, no measureable volatilization loss of the addition agent was found.

## EXAMPLE II

A vinyl plastic sheet 12" x 16" was silvered by a common reduction method and rinsed. It was then placed in a rectangular horizontal cell and clamped into place so that it was one inch above a lead anode of similar size. A solution containing 50 ounces per gallon of nickel sulfate, 6 ounces per gallon of boric acid, and 0.005 gram per liter of acetylamino coumarin at about 150° F. was pumped through the cell at a speed of about 400 feet per minute. The pH of the solution was 3.5 and was maintained at approximately this point by feeding nickel carbonate into an auxiliary tank. Electrolysis was started at 100 amperes per square foot for two minutes and then increased to 1,000 amperes per square foot for nine minutes. The deposit was approximately 7 mils in thickness and was semibright. However, it was burned in some areas.

The same experiment was conducted at 160° F. and 800 feet per minute, and in this instance the nickel deposit was considerably more ductile and no burning was observed.

Utilizing a set of conditions similar to that described in Example II above and utilizing a temperature of 160° F. and 500 feet per minute for the rate of flow of the electrolyte; but employing 0.1 gram per liter of 7-diethyl-

amino-4-methyl coumarin as the addition agent, the deposit was bright-semibright but slightly brittle. The addition of 0.1 gram per liter of trichloroethoxy ethanol made the deposit somewhat brighter and more ductile.

## EXAMPLE III

One gallon of a Watts nickel solution containing 0.2 gram per liter of 3-chlorocoumarin was operated at 160° F. and 600 amperes per square foot for 600 ampere hours with 1½" rotating brass cylindrical cathode having a diameter of 1½". An anode composed of nickel was so configured as to operate at an average current density of 50 amperes per square foot. The addition agent was maintained at 0.2±0.1 gram per liter. At the end of this period, the build-up of the reduction products of the addition agent (principally melilotic acid) had become 0.8 gram per liter. For this reason the nickel deposit was not fully semibright.

An experiment similar to that of Example III in an all sulfate bath was performed and a platinized titanium anode was used; that it, an insoluble anode. As a result the breakdown products of the addition agent reached equilibrium at about 0.2 gram per liter and the deposit was fully semibright.

As stated earlier in the application, the plating bath of the instant invention must be maintained in the pH range of about 2.0 to 4.5. In any plating bath employing the present invention, the bath should be buffered so that the pH remains relatively constant during operation. When operating at pH's above approximately 3.0, it is beneficial to use boric acid to regulate the pH. The presence of the boric acid in addition to affecting pH appears to have an effect on the ductility and brightness of the deposit and is beneficial above a pH 3.0. At a pH of 4.0 and above, boric acid is necessary to eliminate "burning" of the deposit unless the agitation rate is extremely high.

The preferred pH range is between 2.5 and 3.2. Boric acid will not buffer in this pH range and thus it is necessary to utilize an acid having a high buffer capacity in this pH range. Such buffers would include any acid having a pK value of between 2.0 and 4.85. Of course, these same buffering agents could be used at the other pH ranges operable in the instant invention. The concentration of the buffering agent used can vary from approximately 1 to 10 grams per liter depending of course on the extent of use of the bath and the buffering capacity desired. Typical buffers and their buffering concentrations are as follows.

|                                        | G./l. |
|----------------------------------------|-------|
| (1) Monochloroacetic acid -----        | 3     |
| (2) o-Phthalic acid -----              | 4     |
| (3) Dihydroxybenzoic acid (2, 5) ----- | 3     |
| (4) Citric acid -----                  | 5     |
| (5) Hydrofluoric acid -----            | 3     |
| (6) Succinic acid -----                | 4     |
| (7) Acetic acid -----                  | 5     |
| (8) n-butyric acid -----               | 2     |
| (9) o-Hydroxybenzoic acid -----        | 3     |
| (10) Formic acid -----                 | 3     |
| (11) Mandelic acid -----               | 3     |

When operating in the preferred pH range or lower, an additional advantage is obtained by the practice of the instant invention. When operating a chloride free nickel solution such as a nickel sulfate bath with insoluble anodes, the pH drops and the nickel content of the solution also decreases. It is therefore necessary to replenish the nickel and at the same time raise the pH to obtain uniform operating conditions. The nickel supply can be replenished by the use of nickel hydrate, nickel oxide, nickel carbonate, nickel metal powder or electrolytic means using anodes in an auxiliary tank. At a given pH the dissolution rate of nickel hydrate or commercial nickel carbonate is relatively fast compared to nickel oxide or metal. However, the cost of the hydrate

and carbonate is considerably higher than that of the metal or oxide.

It is therefore desirable to operate under conditions which will effect more rapid dissolution of the metal or oxide. The higher the hydrogen ion content (lower pH) the faster the metal or its oxide will dissolve. Therefore, by using the buffers of the instant invention, the pH of the solution is maintained in the pH range wherein the metal and the oxide will readily ionize and there is no need to use the more expansive nickel hydrate or nickel carbonate. Also the buffering agents tend to maintain the pH at the same value and therefore permit easily obtained uniform operating conditions.

To further illustrate the present invention, various examples are given in the following tables using various buffering agents. The operating conditions of the plating bath in the following examples consisted of 52 oz. per gallon of nickel sulfate at a cathode current density of 1,000 amperes per square foot and a temperature maintained at 180° F.

or a substituted coumarin compound in a concentration range of approximately 0.05 to about 0.5 gram per liter. The preferred concentration of the coumarin compounds are between 0.1 and 0.3 gram per liter.

It has been stated earlier in the specification that in the lower pH range buffering agents having a pK value between 2.0 and 4.85 are preferred and should also be pointed out that along with such buffering agents boric acid may be added as a secondary buffer and in such cases the concentration range of the boric acid can vary from preferably 1-3 oz. per gallon.

We claim:

1. A process for the high speed electrodeposition of nickel comprising electrodepositing nickel on a cathode while employing an insoluble anode from a chlorine and bromine ion free bath consisting essentially of an aqueous solution of nickel sulfate having a pH within the range of 2.0 to 4.5 and containing a 1,2-benzopyrone compound, during said electrodeposition said bath being passed at least 300 feet per minute over said cathode at

| Addition Agents                                                                         | pH      | Ductility | Appearance              |
|-----------------------------------------------------------------------------------------|---------|-----------|-------------------------|
| (1) No buffer.....                                                                      | 2.8-2.4 | .05-.15   | Dull S.B.               |
| (2) No buffer.....                                                                      | 4.0     | .....     | Burned and exfoliated.  |
| (3) Boric acid 5 oz./gal.....                                                           | 4.0     | .5        | Grey.                   |
| (4) Boric acid 5 oz./gal.....                                                           | 2.8-2.4 | .05-.15   | Dull S.B.               |
| (5) Boric acid 5 oz./gal. plus .2 g./l. coumarin.....                                   | 2.5     | .5        | S.B. and leveling.      |
| (6) Na citrate 6.8 g./l.....                                                            | 2.5     | .5        | Grey.                   |
| (7) Na citrate 6.8 g./l. plus .2 g./l. coumarin.....                                    | 2.5     | .5        | S.B. and leveling.      |
| (8) Na citrate 6.8 g./l. plus .2 g./l. coumarin.....                                    | 3.8     | .06       | Bt. With sl. burning.   |
| (9) KF-2H <sub>2</sub> O, 2 g./l.....                                                   | 2.5     | .3        | Dull S.B.               |
| (10) KF-2H <sub>2</sub> O, 2 g./l. plus g./l. coumarin.....                             | 2.5     | .5        | S.B. and leveling.      |
| (11) KF-2H <sub>2</sub> O, 2 g./l.....                                                  | 3.3     | .5        | Bt. S.B. and leveling.  |
| (12) KF-2H <sub>2</sub> O, 2 g./l.....                                                  | 3.8     | .04       | Do.                     |
| (13) KF-2H <sub>2</sub> O, 2 g./l plus 3 oz./gal. H <sub>3</sub> BO <sub>3</sub> .....  | 3.8     | .5        | Do.                     |
| (14) 2,5 dihydroxybenzoic acid.....                                                     | 2.5     | .5        | S.B.                    |
| (15) 2,5 dihydroxybenzoic acid plus .2 g./l. coumarin.....                              | 2.5     | .5        | S.B. and leveling.      |
| (16) 2,5 dihydroxybenzoic acid plus .2 g./l. coumarin.....                              | 3.8     | .08       | Bt. S.B. with burning.  |
| (17) Acetic acid 2 cc./l.....                                                           | 2.5     | .4        | S.B.                    |
| (18) Acetic acid 2 cc./l plus .2 g./l. coumarin.....                                    | 2.5     | .5        | S.B. and leveling.      |
| (19) o-Phthalic acid 3 g./l.....                                                        | 2.5     | .5        | Grey.                   |
| (20) o-Phthalic acid 3 g./l plus .2 g./l. coumarin.....                                 | 2.5     | .5        | S.B. and leveling.      |
| (21) o-Phthalic acid 3 g./l. plus 2 g./l. coumarin plus 2.5 g./l. butynediol.....       | 2.5     | .5        | Bt. S.B. leveling.      |
| (22) Boric acid 5 oz./gal. plus .25 g./l. butynediol.....                               | 2.5     | .07       | Bt. S.B.                |
| (23) n-Butyric acid 4 g./l.....                                                         | 2.5     | .5        | S.B.                    |
| (24) n-Butyric acid 4 g./l. plus .2 g./l. coumarin.....                                 | 2.5     | .5        | S.B. and leveling.      |
| (25) Formic acid 3 cc./l.....                                                           | 2.5     | .25       | S.B.                    |
| (26) Formic acid 3 cc./l. plus .2 g./l. coumarin.....                                   | 2.5     | .5        | S.B. and leveling.      |
| (27) Ni(BF <sub>4</sub> ) <sub>2</sub> , 4.0 g./l.....                                  | 2.6     | .07       | Bt. S.B.                |
| (28) Ni(BF <sub>4</sub> ) <sub>2</sub> , 4.0 g./l. plus .2 g./l. coumarin.....          | 2.6     | .5        | Bt. S.B. and leveling.  |
| (29) KF-2H <sub>2</sub> O, 2 g./l.....                                                  | 2.5     | .3        | Dull S.B.               |
| (30) KF-2H <sub>2</sub> O, 2 g./l. plus .1 g./l. butynediol.....                        | 2.5     | .25       | S.B. with leveling.     |
| (31) KF-2H <sub>2</sub> O, 2 g./l. plus .1 g./l. butynediol plus .2 g./l. coumarin..... | 2.5     | .35       | Bt. S.B. with leveling. |
| (32) o-Phthalic acid 3 g./l.....                                                        | 2.5     | .5        | Grey.                   |
| (33) o-Phthalic acid 3 g./l. plus .2 g./l. of 6-acetamide coumarin.....                 | 2.5     | .5        | S.B. with leveling.     |

In the ductility values given in the above table, the value .5 indicates .5 or better; S.B. indicates semi-bright; Bt. indicates bright and sl. indicates slight.

As can be noted from the examples given in the above table in addition to the presence of coumarin and a buffering agent, certain unsaturated compounds may also be included in the plating bath and result in brighter electroplate. Typical such unsaturated materials include bis-( $\beta$ -hydroxyethoxy butyne-2), diethyleneglycolmonopropargyl ether and butynediol-1,4. These materials may be present in a concentration from about 0.005 to 0.5 gram per liter. The preferred concentration of the butynediol is between about 0.2 and 0.3 gram per liter with a maximum utility appearing at a concentration of .25 gram per liter. The bis-( $\beta$ -hydroxyethoxy butyne-2) and diethyleneglycolmonopropargyl ether are present preferably in concentrations from 0.1 to 0.3 grams per liter. Maximum brightening appears when using bis-( $\beta$ -hydroxyethoxy butyne-2) at a concentration of about 0.1 gram per liter while with diethylene glycolmonopropargyl ether maximum brightening appears to coincide with a concentration of 0.15 gram per liter. Such concentration of these additional brightening agents may be added to the plating bath of the instant invention which contains a coumarin

a current density of at least 500 amperes per square foot and at a temperature of at least 150° F., said compound having a boiling point greater than about 290° C. and a melting point greater than about 70° C.

2. A process for the high speed electrodeposition of nickel comprising electrodepositing nickel on a cathode while employing an insoluble anode from a chlorine and bromine ion free bath having a pH within the range of 2.0 to 4.5 consisting essentially of an aqueous solution of nickel sulfate and containing an addition agent selected from the group consisting of 3-chlorocoumarin, 3-acetylcoumarin, -6-acetylaminocoumarin, 3-hydroxy-coumarin, 3-cyanocoumarin, 3- or 4-methyl coumarin, 6-methyl coumarin, 4,8-dimethyl coumarin, 7-diethyl-amino-4-methyl coumarin, 6-hydroxycoumarin, 6-(1-glucosaminio) coumarin, 6-hydroxymethyl coumarin, 8-hydroxyethyl coumarin, 7-methoxycoumarin, and 8-ethoxycoumarin, during said electrodeposition said bath being passed at least 300 feet per minute over said cathode, at a current density of at least 500 amperes per square foot at a temperature of at least 150° F.

3. A process for the high speed electrodeposition of nickel comprising electrodepositing nickel on a cathode while employing an insoluble anode from a chlorine and

bromine ion free bath having a pH within the range of 2.0 to 4.5 consisting essentially of an aqueous solution of nickel sulfate and containing an addition agent selected from the group consisting of 0.0002 to 0.003 mole per liter of 3-chlorocoumarin, 0.0002 to 0.003 mole per liter of 3-acetylcoumarin, 0.0002 to 0.002 mole per liter of 3-hydroxycoumarin, 0.0002 to 0.002 mole per liter of 6-acetylaminocoumarin, 0.0002 to 0.002 mole per liter of 3-cyanocoumarin, 0.0002 to 0.003 mole per liter of 3- or 4-methyl coumarin, 0.0002 to 0.003 mole per liter of 6-methyl coumarin, 0.0002 to 0.003 mole per liter of 4,8-dimethyl coumarin, 0.0002 to 0.002 mole per liter of 7-diethylamino-4-methyl coumarin, 0.001 to 0.004 mole per liter of 6-hydroxycoumarin, 0.0002 to 0.002 mole per liter of 6-(1-glucoseamino) coumarin, 0.0002 to 0.003 mole per liter of 6-hydroxymethyl coumarin, 0.0002 to 0.003 mole per liter of 8-hydroxyethyl coumarin, 0.0002 to 0.003 mole per liter of 7-methoxycoumarin, and 0.0002 to 0.003 mole per liter of 8-ethoxycoumarin, said bath being subject to high agitation so that the bath is rapidly passed over the surface of the cathode at a rate equivalent to at least 600 feet per minute, is supplied at a current density of at least 500 amperes per square foot and a temperature of at least 150° F.

4. A process for the high speed electrodeposition of nickel comprising electrodepositing nickel on a cathode while employing an insoluble anode from a chlorine and bromine ion free bath having a pH within the range of 2.0 to 4.5 consisting essentially of an aqueous solution of nickel sulfate and containing an addition agent selected from the group consisting of 0.0002 to 0.003 mole per liter of 3-chlorocoumarin, 0.0002 to 0.003 mole per liter of 3-acetylcoumarin, 0.0002 to 0.002 mole per liter of 6-acetylcoumarin, 0.0002 to 0.002 mole per liter of 3-hydroxycoumarin, 0.0002 to 0.002 mole per liter of 3-cyanocoumarin, 0.0002 to 0.003 mole per liter of 3- or 4-methylcoumarin, 0.0002 to 0.003 mole per liter of 6-methyl coumarin, 0.0002 to 0.003 mole per liter of 4,8-dimethyl coumarin, 0.0002 to 0.002 mole per liter of 7-diethylamino-4-methyl coumarin, 0.001 to 0.004 mole per liter of 6-hydroxycoumarin, 0.0002 to 0.002 mole per liter of 6-(1-glucoseamino) coumarin, 0.0002 to 0.003 mole per liter of 6-hydroxymethyl coumarin, 0.0002 to 0.003 mole per liter of 8-hydroxyethyl coumarin, 0.0002 to 0.003 mole per liter of 7-methoxycoumarin, and 0.0002 to 0.003 mole per liter of 8-ethoxycoumarin, said bath being passed over the surface of the cathode at a rate of at least 600 feet per minute at a current density in excess of 1,000 amperes per square foot and at a temperature in the range of about 180 to 210° F.

5. A process for the high speed electrodeposition of nickel comprising electrodepositing nickel on a cathode while employing an insoluble anode from a chlorine and bromine ion free bath having a pH within the range of 2.0 to 4.5 consisting essentially of an acidic aqueous solution of nickel sulfate and containing a 1,2-benzopyrone compound having a boiling point greater than 290° C. and a melting point greater than about 70° C., said electrodeposition being further characterized in that the bath is subject to high agitation such that a flow rate at the cathode of at least 300 feet per minute is produced and the current density at the cathode is at least 500 amperes per square foot and the bath temperature is at least 150° F.

6. A process for the high speed electrodeposition of nickel comprising electrodepositing nickel on a cathode while employing an insoluble anode from a chlorine and bromine ion free bath consisting essentially of a buffered aqueous solution of nickel ions having a pH within the range of 2.0 and 4.5 and containing a 1,2-benzopyrone compound, said buffering being produced by a buffer effective in the pH range of 2.0 to 4.0, during said

5 electrodeposition said bath being passed over said cathode at a rate of at least 300 feet per minute while employing a current density of at least 500 amperes per square foot and operating said bath at a temperature of at least 150° F.

10 7. A process for the high speed electrodeposition of nickel comprising electrodepositing nickel on a cathode while employing an insoluble anode at current densities of at least 500 amperes per square foot at the cathode under high agitation conditions wherein the flow rate past the cathode is at least 300 feet per minute from a chlorine and bromine ion free bath consisting essentially of an aqueous solution of nickel ions having a pH within the range of 2.5 to 3.2 and containing a 1,2-benzopyrone compound along with a buffering agent capable of buffering said bath in the pH range of 2.5 to 4.0 which has a pK value in the range of 2.0 to 4.85, said bath being maintained during said electrodeposition at a temperature of at least 180° F.

15 20 8. A process for the high speed electrodeposition of nickel comprising electrodepositing nickel on a cathode while employing an insoluble anode at current densities of at least 500 amperes per square foot at the cathode under high agitation conditions wherein the flow rate past the cathode is at least 300 feet per minute from a chlorine and bromine ion free bath consisting essentially of an aqueous solution of nickel ions having a pH within the range of 2.5 to 3.2 and containing between about 0.05 and 0.5 gram per liter of a 1,2-benzopyrone compound along with from 1 to 10 grams per liter of a buffering agent capable of buffering said bath in the pH range of 2.5 to 4.0 which has a pK value in the range of 2.0 to 4.85, said bath being maintained during said electrodeposition at a temperature of at least 180° F.

30 35 9. A process for the high speed electrodeposition of nickel comprising electrodepositing nickel on a cathode while employing an insoluble anode at current densities of at least 500 amperes per square foot at the cathode under high agitation conditions wherein the flow rate past the cathode is at least 300 feet per minute from a chlorine and bromine ion free bath consisting essentially of an aqueous solution of nickel ions having a pH within the range of 2.5 to 3.2 and containing 0.1 to 0.3 gram per liter of a 1,2-benzopyrone compound, 1 to 10 grams per liter of a buffering agent capable of buffering said bath in the pH range of 2.5 to 4.0 which has a pK value in the range of 2.0 to 4.85 and between about 0.005 and 0.5 gram per liter of a compound selected from the group consisting of bis-( $\beta$ -hydroxyethoxy butyne-2), diethylene-glycolmonopropargyl ether and butynediol, said bath being maintained during said electrodeposition at a temperature between 180° F. and 210° F.

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 913

UNITED STATES PATENT OFFICE  
CERTIFICATE OF CORRECTION

Patent No. 3,488,264

January 6, 1970

Raymond E. Bailey et al.

It is certified that error appears in the above identified patent and that said Letters Patent are hereby corrected as shown below:

Column 7, line 10, "expansive" should read -- expensive --; same column 7, addition agent No. 21, should read -- o-Phthalic acid 3 g/l plus .2 g/l coumarin plus .25 g/l butynediol --. Column 9, line 15, 0,0002" should read -- 0.0002 --; line 34, "6-acetylcoumarin" should read -- 6-acetylaminocoumarin --.

Signed and sealed this 10th day of November 1970.

(SEAL)

Attest:

Edward M. Fletcher, Jr.

Attesting Officer

WILLIAM E. SCHUYLER, JR.

Commissioner of Patents